

## UNITED STATES PATENT OFFICE

2,127,533

METHOD AND MEANS FOR FOUNDRY  
PRACTICE

Charles Marshall Saeger, Jr., Bowmanstown, Pa.

No Drawing. Application January 12, 1929,  
Serial No. 332,225

6 Claims. (Cl. 22—188)

(Granted under the act of March 3, 1883, as  
amended April 30, 1928; 370 O. G. 757)

My invention relates to a new and useful method of making molds and cores for metal castings.

Previously in this art the hot metal coming in contact with the mold and core surfaces causes the sand in contact to burn into the adjacent surfaces of the metal and produces castings of rough exterior and interior surfaces, which surfaces are formed of an integral film of mixed metal and sand. This, as well as the removal of the cores and the cleaning of the un-integral sand from the casting, has heretofore been an expensive, laborious and dusty task frequently requiring the use of pneumatic chisels and other tools, while in the machining of such castings the integral film of sand and metal is difficult to machine unless the tool in its first cut penetrates beyond the depth of such film.

In the prior art many cracked castings have been produced due to hard cores and molds which do not crush readily as the metal casting cools, contracts and solidifies, and such castings are a constant source of substantial loss in all foundries but more especially in aluminum and kindred metal castings.

A further constant source of substantial loss in the prior art of metal casting has resulted from mold and core blows due to the low permeability of the sand forming such molds and cores.

In the past many endeavors have been made to overcome these very objectionable conditions and losses. Some of these attempts have been to form the molds and cores of green sand, which is the ordinary molding sand of commerce, but the liability of such molds and cores to be washed in part into the molten flowing metal being cast prevents, or renders hazardous, their use in many cases.

To provide molds and cores of more strength than possessed by green said molds and cores, it heretofore has been common practice to embody a binder in the sand of, either or all, clay, molasses and water, flour and water, and oil, and to indurate such molds and cores by baking. Such molds and cores have all the aforesaid defects except the tendency to wash into the flowing molten metal, while the thus formed harder molds and cores increase the cracking liability of the castings as well as tend to increase the liability of the castings to blow due to the lesser porosity of such molds and cores.

In the prior art water has been employed as a diluent of the active binding material employed but its surface tension, rate of evaporation and other conditions, are such that it requires sub-

stantial labor in order to properly mix the same with the constituent material of the mold or core, while its vaporizing point is so high as to leave much of the water in the mold or core or requires that such mold or core be baked sufficiently to remove such moisture, which baking to the degree required to remove such moisture produces a hard core or mold with its said liabilities.

In the overcoming of the aforesaid conditions and losses I have devised a method of producing molds and cores for metal castings which contemplates the addition to the sand forming such molds and cores, either or both, rubber or a rubber-like substance in solution or dispersion which may be mixed throughout the whole mass of such molds and cores or the surface of the mold or core or both that comes in contact with the metal to be cast may be impregnated with such rubber or rubber-like substance in solution or dispersion. The solution being formed by any desirable solvent of rubber or rubber-like material, or said dispersion being formed by small particles thereof in a liquid, and such solvent or liquid is preferably of the class that may readily be evaporated so that a further step in my method, that of drying the mold or core may readily be accomplished either by atmospheric temperature or by moderate heat as the element of time or other production factors may determine to be most economic or desirable. When the molds, and such cores as they may have, are thus dried the molten metal may be cast therein and the heat of such cast metal in contact with the surfaces of the molds, as well as of such cores that they may contain, causes the rubber or rubber-like binder to be destroyed by said application of said heat. Said destruction, disintegration or the loss of its binding efficiency, does not take place until a predetermined time after the molten metal has been poured in the mold and/or about the core, said time being after the process of solidification of the cast metal, or at least the surfaces thereof juxtaposed to the mold and/or core, has rendered such metal, or said surfaces thereof, not fluid, as otherwise the casting would be liable to be rendered defective or useless by the particles of the mold and/or core, which are by the heat of said casting no longer bound together, being washed into or becoming commingled or imbedded in the casting. In the said application of said heat to the exposed surfaces of the mold, and core or cores that the mold may contain, the presence of rubber or rubber-like material causes the surfaces of the metal not to burn in or inter-

mingle with substantially any of the sand as it does in the prior art.

As to this last named phenomenon, applicant has not yet been able to learn the agencies which produce this end. He has with his associates accounted for said phenomenon on two theories either or both of which may explain the existence of said phenomenon.

One of said theories is that the hot surface of the casting in contact with the rubber impregnated sand mold and core forms a gaseous layer adjacent to the hot metal surfaces which prevents the sand adhering to or being embedded into the hot metal surfaces.

15 The other theory being that such hot metal in contact with such rubber-like impregnated sand results in the formation of free carbon which coats the grains of sand and thereby prevents such coated sands from either directly 20 coming in contact with or being embedded in the surface of the casting.

It has further been found that the grains of sand forming the mold and the cores that have been impregnated or mixed with said rubber or 25 rubber-like material are, due to the heat of the casting, coated with decomposition products of rubber occasioned by the conversion of said rubber or rubber-like material, and this condition is believed to be the main or contributing factor 30 in rendering especially the cores to be most readily removed from all castings; whereas in the prior art it has been the usual custom of requiring as much as a day for the removal of some cores from a single casting with the best labor 35 saving appliances.

In order to demonstrate the practical utility of my said method I have caused many molds and cores to be constructed in accordance with my said method and in so constructing the same 40 I have formed a rubber or rubber-like solution embodying for instance 1 lb. of rubber or rubber-like substance dissolved in 2 gallons of gasoline and have therewith moistened or tempered the dry sand to the usual or required molding consistency. From such moistened or tempered sand I have caused the molds and cores to be 45 formed. Then I have dried such molds and their required cores, if any, either by atmospheric temperature or by the application of moderate heat thereto according to convenience or the production speed required. When dried the casting 50 may be made in the assembled mold with the cores therein that may be required.

Under favorable conditions where the strength 55 of the ordinary green sand mold or core would be 2.4 lbs. per square inch, my said method of producing a mold or core results, for instance, in the same having a corresponding strength 60 of 10.8 lbs. per square inch and yet the permeability of my sand molds and cores is as great as, if not greater than, the green sand molds and cores so that practically no castings are lost from the blowing of either molds or cores. However, I have, by my said method or process, produced molds and cores at atmospheric temperatures 65 of greater strength than baked molds and cores, but when subjected to the casting heat they are of greater gas permeability and yieldability, to casting shrinkage, by employing, different proportions of solvent and rubber or 70 rubber-like material, or less of the elastic and more of the plastic properties of such materials.

In the old art where great difficulty has always been experienced in removing cores from castings, some of which have to be virtually chipped

out a piece at a time, my method wherein the heat destroys the binder, renders the cores granular and free flowing as dry sand. In the old art where clay and other binders were used which when burnt by making one casting could not be used with molding sand to form the exterior surfaces of the mold, with my method, in removing the casting from the mold the core sands will shake out of the core holes and mingle with the exterior surface molding sands which, with my 10 method, is unobjectionable because even any core sands may be reused while in the prior art core sand that has been previously used in making a casting of molten metal could not be reused for any molding purpose except to form 15 partings.

In practice many characters and weights of castings of many different metals and their alloys are required to be made and in the production of some of these castings it may be found convenient 20 or desirable to increase or decrease the amount of rubber or rubber-like or plastic material employed as well as to employ other well-known solvents other than gasoline. Some of these well-known solvents are objectionable due to their 25 toxic effect upon the personnel while others are objectionable in usual production due to their substantially higher rate of evaporation as their employment renders difficult the even distribution of such solvents with their rubber content 30 throughout the sand unless such sand be mixed therewith under conditions in excess of atmospheric pressure or with greater than normal rapidity.

While it has been stated that the rubber or 35 rubber-like substance or material has been reduced to the form of a solution before the sand is applied to or commingled with the material forming the mold or core, yet this is only one of the convenient ways for obtaining such a mixture. Another of such ways being that the rubber or 40 rubber-like material or substance is reduced to a granular or powdered form and directly mixed in such condition with the sands or other material forming the mold or core. The interlocking 45 characteristics of such a mixture in practice may afford the requisite bond, but in such cases where the shape or weight or other characteristics of the mold or core may not be thus afforded the requisite bonding capacity, such capacity may be 50 substantially increased by the application to the mass of a moderate degree of heat and pressure, either or both.

A further beneficial accomplishment of my invention is that it enables castings to be produced 55 without oxidized surfaces so that the bright un-oxidized surfaces of the cast metal appear when removed from the mold. This produces a casting of better appearance and tends substantially to deter subsequent oxidizing tendencies. This is 60 more especially advantageous in producing castings of the more readily oxidizable metals as well as with such castings having relatively thin portions which are not required to be finished. Furthermore, such molds and their cores, and the 65 heat action of the molten metal thereon tend to avoid any harmful action upon the casting and its surface that may be set up in the other than rubber or rubber-like material content of the mold and core.

In the binders of the prior art with which water 70 has been present in the molds or cores or has been employed as a diluent, it is the theory that, when the hot metal is cast into or against molds or cores bonded with such binder, the heat of the 75

liquid metal vaporizes the water content of the mold or core relatively slowly and fills the cavity of the mold with water vapor which oxidizes the surface of the metal and which water vapor or gas tends to prevent the charring of the organic substances on the mold and core surfaces and thus causes contact of said oxidized surfaces of the cast metal with the uncoated or uninsulated sand grains, and which results in the fusing, imbedding into or adherence of said sand to the surfaces of the casting. This action also leaves a substantial oxygen content, residual from the air, in the casting-cavity of the mold, which is being filled with the hot liquid metal, and which oxygen also promotes oxidation of the metal surfaces and the removal of said char from the mold or core surfaces, thus contributing to said fusing of and adherence to the casting surfaces.

In the binder which I employ with a diluent whose volatility is substantially greater than water, and which contains substantially less oxygen, the theory is that when the hot metal is cast into or against molds or cores bonded with such binder, the heat of the liquid metal vaporizes said diluent relatively more rapidly and quickly forms a gas or vapor which expels or replaces the air content of the cavity of such mold, and which gas or vapor thus formed is in itself more free from oxygen than water vapor. These conditions, namely, the substantial absence of air and the occupation of said cavity by a reducing or non-oxidizing gas or vapor, promote the charring of the binder upon the mold or core surfaces, tend to prevent the removal of such charred coating by oxidation or combustion, and thus preclude the fusion or adherence of the mold or core particles with or to the surfaces of the casting.

Upon said conditions in the prior art, and in my invention, the prior art castings are formed in the presence of an oxidizing gas or vapor, while in my invention the castings are formed in the presence of a non-oxidizing gas or vapor.

The active constituent which I employ as a binder should, I have discovered, be sparingly present in the parts of the mold or core at, or close to, the surface of the hot casting and should be prevented from collecting or accumulating at or near any such surface, as, under the aforesaid theory of the action of my invention, said active constituent upon the casting-surface of the mold or core is of such low charring temperature that it may char before the cast metal fills the mold, whereby the lighter of the thus combusted gases may escape from the mold which is ventilated by the usual poring and riser grates until the casting-cavity of the mold becomes full of cast metal. Such char is only required to be thin to prevent the material forming the mold and core from being imbedded in, or adhering to, or fusing with the surface of the casting. The constituent material of the mold or core requires but little of said active constituent of my binder to bind said material. Thus, in respect to obtaining said surface char as well as said binding economy in the use of said active constituent is not only desirable but is in many cases productive of the best results. The presence in the mold at the time of the casting therein, of the non-oxidizing gas or vapor tends to prevent the removal of such char and promotes said economy, since the sparing amount of char-producing substance upon such surfaces that is originally placed there remains to prevent the fusion of the mold or core particles with the surfaces of the casting.

In order to economically attain said results, I

dilute or weaken the normal strength of said active constituent by admixture with another substance, all ingredients of such mixture being preferably either in powdered or liquid form before or after such admixture.

In order to obtain the most economical results in a liquid form of said active constituent a liquid diluent is employed whose surface tension is substantially less, and whose rate of evaporation is substantially higher, and whose other qualities are substantially more favorable than those of water. For instance, when a drop of water is placed on an impervious surface, force is required to spread said drop over said surface due, in part, to the high surface tension of water; but when a fluid of substantially lesser surface tension is, for instance, dropped upon such a substance, such fluid more readily spreads over a wide area of such surface. While capillary action has some tendency to decelerate such spread over a pervious surface of the same substance, the problem in an economical core binder is to have the binding fluid quickly spread over the external surface of the particles of the substance to be bonded together, as the fluid absorbed by capillary action into the pores of such particles is substantially wasted from a binder sense. Thus, I have discovered, that the requisite dilution of the active constituent of my binder by a fluid of substantially lower surface tension, and whose rate of evaporation is substantially higher, and whose other qualities are more favorable, than those of water also greatly facilitates the spreading of said binder over the outer surfaces of the particles of the material comprising the molds and cores and substantially lessens the labor of mixing said binder with said material, and whose loss due to capillary action is substantially less and more economical. The substantial decrease over water of the volatility of said fluid diluent enables the same to be readily evaporated from the molds and cores, even by air drying, before castings are formed therewith.

In this specification and its appended claims where the term, rubber, is employed it is intended to include rubber either as latex, coagulated rubber, or sap from trees such as *Hevea brasiliensis*, or from vines or shrubs, as well as from other kindred vegetation such as guayule containing more or less rubber hydrocarbon. The rubber may be unvulcanized or consist of vulcanized soft rubber, and may have been previously subjected to an elevated temperature.

By rubber-like material employed in the specification and its appended claims it is desired to be understood as referring to any substance, either or both plastic and elastic, that have any of the substantial characteristics of rubber, balata or gutta percha, and may include old rubber scrap that has been treated either at an elevated temperature alone or otherwise. It may also include any rubber or scrap rubber, either or both, that has been subjected to an elevated temperature alone or in the presence of sulphuric acid or a sulphonic acid or a sulphonyl halide or it may also include a substance such as is an article of commerce under the name "Thermoprene".

The invention herein described may be manufactured and used by or for the Government of the United States for governmental purposes without the payment to me of any royalty thereon or therefor.

As to certain features set forth in the foregoing specification see also my copending applications

Serial No. 332,226, filed January 12, 1929, for "Process and product for coating molds and cores", and Serial No. 429,227, filed February 17, 1930, for "Method and means for foundry practice".

- Having now so fully described my invention that others skilled in the art may therefrom make and use the same, what I claim and desire to secure by Letters Patent is:
10. 1. In the method of producing cores and molds, the step of mixing with component material of such molds and cores rubber in divided particles adapted to be combusted by the heat of the casting.
  15. 2. In the method of producing cores and molds, the step of mixing with the material for the entire body of such molds and cores rubber in solution.
  20. 3. The method of making a core for metal castings consisting in mixing a quantity of sand with a binder including a thermoprene cement of the G. P. type, forming a core from such mix-

ture, and permitting the core to cure in contact with the air.

4. A core material for sand cores comprising an aggregate and a solution of a thermoprene of the gutta-percha type as a binder.

5. A core binder for foundry refractory substances comprising a solvent, volatile at room temperatures, containing an adhesive rubber compound having the physical characteristic of disintegrating into granular carbon within the range of temperature to which the refractory substance is to be subjected during the cooling of the cast metal.

6. A casting mold or core for metal casting comprising a granular refractory substance bound together throughout with an adhesive rubber compound having the physical characteristic of disintegrating into granular carbon within the range of temperatures to which the mold or core is to be subjected during the cooling of the cast metal.

CHARLES MARSHALL SAEGER, JR.